

## UNITED STATES PATENT OFFICE

1,935,588

## LUBRICATING COMPOUND

Samuel Cabot, Jamaica Plain, Mass., assignor to  
 Polygon Products Company, Boston, Mass., a  
 corporation of Massachusetts

No Drawing. Application May 31, 1932  
 Serial No. 614,645

11 Claims. (Cl. 87-9)

In the lubrication of surfaces working in close contact where continuous feed may not be had or is difficult to establish or maintain, there has been a recognized need of lubricating materials 5 which would reach the most inaccessible of these surfaces and yet be effective upon reaching such areas.

In newly assembled parts, as in engine pistons, 10 bearings and valves, as well as in spring leaves or like assemblies, the immediate and recurrent problem is that of the penetration of a highly lubricating medium which will not only make possible the process of the wearing in of the new moving parts, but will establish surface conditions 15 maintainable by ordinary lubrication of these parts after use.

The difficulty is to get highly efficient lubrication into remote or tightly fitting parts. Furthermore, the problems being various require 20 in any commercial solution a product which will function under the various conditions and give the results desired.

The object of my invention is to produce a new material for this type of penetrating lubrication. 25 A penetrating lubricant must have as low a degree of viscosity as practicable in order to penetrate, but at the same time must contain as great a proportion of the best possible lubricant as can be compounded in it.

According to my invention the best composition 30 for penetrating lubrication should consist of a high grade lubricant which has been further improved by addition of a comparatively small percentage of a material colloidally dispersable in it, and the viscosity lowered by addition of pre-determined quantities of a thinning material of 35 low viscosity, preferably of a volatile character, in which the lubricant is soluble and the colloid colloidally dispersable.

According to my concept the most suitable colloid 40 to be used in conjunction with certain lubricants in this composition is a substance which is an isomer or polymer of the lubricant. A composition in which the colloid is an isomer or polymer of the lubricant shows less increase of viscosity (due to internal friction) and more slip 45 than when other colloids are used.

There are definite limits within which this applies. 50 It applies substantially only to such lubricants as those made from paraffin, naphthene and olefin hydrocarbons or from semi-drying or hydroxy animal or vegetable oils or greases.

For instance, a mixture of olefin hydrocarbons 55 whose average empirical formula is  $C_{20}H_{40}$  may be polymerized by known means to products

whose average empirical formula is  $C_{40}H_{80}$ ,  $C_{50}H_{100}$ , etc., and which are colloidally dispersable in the original hydrocarbon. It is a general characteristic for an isomer to be more readily dispersable in its isomer than a non-isomer. Furthermore, polymers are more readily dispersable when they are derived from the same or original starting material. In other words, a polymer usually has greater dispersability in the monomer from which it is derived.

Materials colloidally dispersable in their isomers or polymers are called isocolloids.

In carrying out the present invention, a material having good lubricating properties has added thereto a relatively small proportion of a polymer thereof, the same being isocolloidally dispersable in the original lubricating material. The preferred lubricating starting material is petroleum oil from which the lighter components such as gasoline, naphtha, kerosene, polar oil, and gas oil have been removed by distillation. Petroleum lubricating oils are generally identified by the character of the base from which they are produced, and are known as paraffin base, naphthene base, or olefin base oils. Lubricating oil mixtures of this character may be improved in accordance with the present invention by isocolloidally dispersing therein a small proportion of polymers thereof. There is preferably added to

the so treated oil an anti-oxidant, and the resulting product is then thinned out to a low viscosity with an appropriate thinning agent. In some cases a polar and/or amphoteric compound may be added. Compounds of an amphoteric character have acid and basic radicals and function as a buffer in the lubricant. A polar compound which is not amphoteric in itself may become amphoteric on coming in contact with the surface lubricated, and the formed amphoteric compounds will assert a buffering action during the

course of lubrication, which is of course eminently desirable. The polar compound may also react with constituents present in the lubricating oil, for example alkali, to form an amphoteric compound asserting a buffering action. The presence of fatty acids or equivalent compounds is also desirable, since they form in situ metallic soaps which lower the surface tension of the

final lubricant.

Although the present invention is particularly 105 satisfactory for treatment of petroleum oils of the character set forth, it may be used in connection with other organic lubricants, and particularly the semi-drying oils and the hydroxy animal or vegetable oils or greases. For ex-

ample, castor oil, whale oil, sperm oil, and the like, yield satisfactory final lubricants when there is added thereto a small proportion of a polymerization product thereof.

5 It may be stated that if a mixture of petroleum oils or other oils are used, then the polymerized product which is added in a small proportion is a polymerized mixture of the original starting materials.

10 Suitable anti-oxidants, these being compounds which inhibit oxidation, are aniline, alpha or beta naphthol, diphenyl-guanidine, hydroquinone, cresylic acid and similar products.

As stated, any desirable polar substances may 15 be added to the lubricant, such substances having unrelated radicals in asymmetric positions which tend to cause orientation of the molecule in relation to a surface or boundary. Any suitable polar substance may be used, and as examples, the following are set forth: fatty acids, such as oleic acid; alcohols, such as cholesterol; esters, such as olein and the like, or mixtures thereof.

Animal grease and sheep grease, the latter being 20 known as degras, are mixtures of fatty esters, fatty acids, and fatty alcohols. Degras or sheep or wool grease, is a very satisfactory polar compound, and in addition has a high lubricating value. Oleic acid may be used as a polar compound, but its lubricating value is relatively low. Castor oil and whale oil are examples of polar compounds which are good lubricants. The only limits to the use of polar compounds of the above character is good practice. These polar compounds which are not hydrocarbons are more 30 chemically active than hydrocarbons and are, therefore, not so good for certain types of lubrication, and obviously the more that is used, the less hydrocarbon lubricant can be used. Where 35 hydrocarbon lubricants are used, the polar compounds which are added should, in the preferred form of the invention, be present in a quantity substantially less than the hydrocarbon lubricant. When using a petroleum base as the lubricant and adding a polymer thereto, about 7% of a polar material such as degras may be added, based on the weight of the hydrocarbon lubricant.

Castor oil, polymerized by heating may be isocolloidally dispersed in castor oil, and similarly cotton seed oil polymerized by heating may be isocolloidally dispersed in cotton seed oil, the polymerized compound being present in the lubricant in a relatively small proportion. As 55 stated, lubricants of this character may be made in accordance with the present invention instead of lubricants derived from hydrocarbons having a paraffin, olefin, or naphthene base. Aromatic hydrocarbons, typified by the coal tar series, those having anthracene and naphthalene oils present, or phenols and bases derived from the coal tar series are not satisfactory for treatment in accordance with the present invention, since such aromatic compounds in their original state are 60 poor lubricants and when they are polymerized or are condensed, form resins and pitches which are largely super-cooled liquids and not colloidally dispersable. Further, such super-cooled resinous and pitch like substances are detrimental to lubrication, and additionally contain large quantities of crystalline materials which are incapable of separation, and therefore render the entire mass solid or pasty at low temperatures. In other words, the aromatic hydrocarbons typified by the coal tar series are known

to yield lubricating agents of a very inferior quality, being more or less lacking in adhesive properties, which of course is essential in a good lubricating agent. It is, therefore, clear that the aromatic hydrocarbons of the coal tar series 8 cannot be used for the original lubricating base, and cannot be satisfactorily polymerized to form a body which is suitable for isocolloidial dispersion in the original lubricating base. However, it is desired to point out that the petroleum bases having hydro-aromatics present, and particularly the naphthenes which are usually present in Caucasian oils and in Louisiana oils, may be treated in accordance with the present invention.

It is essential that my product shall have as 90 low viscosity as produced in order to allow it to penetrate effectively. While of course the viscosity of the final lubricant may vary somewhat, in general the viscosity should not, in the preferred form of the invention, be greater than 6° Engler at 100° F., and preferably much lower. 95

While the following examples are illustrative of the invention, the latter obviously is not limited thereto.

#### Example I

|                                              | Parts by weight |
|----------------------------------------------|-----------------|
| Polymerized olefin or naphthene hydrocarbons | 3               |
| Olefinic or naphthenic lubricating oil       | 30              |
| Oleic acid                                   | 2               |
| Aniline                                      | 1               |
| Mineral naphtha                              | 64              |

#### Example II

|                        | Parts by weight |
|------------------------|-----------------|
| Polymerized castor oil | 3               |
| Castor oil             | 30              |
| Alpha-naphthol         | 1               |
| Solvent naphtha        | 66              |

#### Example III

|                       | Parts by weight |
|-----------------------|-----------------|
| Polymerized whale oil | 2               |
| Whale oil             | 32              |
| Diphenyl-guanidine    | 1/4             |
| Turpentine            | 65 1/4          |

#### Example IV

|                          | Parts by weight |
|--------------------------|-----------------|
| Paraffin lubricating oil | 32              |
| Polymerized paraffin oil | 3               |
| Cresylic acid            | 1               |
| Degras                   | 6               |
| Mineral oil              | 58              |

In any of these the anti-oxidant such as aniline, cresylic acid, alpha-naphthol, diphenyl-guanidine, are interchangeable, as are the penetrants 135 solvent naphtha, mineral naphtha and turpentine. Also to some extent this is true of the polar substances, such as oleic acid, castor oil, degras and whale oil. In the case of castor oil and whale oil they act as lubricants and their polymers as isocolloids, and as polar substances, being of that chemical nature. The hydrocarbons, being non-polar, have added thereto polar substances in the form of degras or oleic acid.

A characteristic compound in accordance with 145 my invention may be made by taking 35% of a petroleum oil of lubricating character, which in this instance may be considered as of an asphaltic base. To this I add 5% of such an asphaltic body as the polymerized residuum available in still 150

bottoms and which are therefore iso-colloidal as regards the petroleum selected. Where an asphaltic iso-colloid is used I preferably add 1% or 2% of aniline oil, as an anti-oxidant as it reduces its gumming tendency. I also preferably add 5% of some animal grease, preferably of polar character, as for example, degras.

Besides still bottoms, hydrocarbons may be readily polymerized by many substances, such as anhydrous aluminum chloride, anhydrous zinc chloride, anhydrous ferric chloride, concentrated sulphuric acid, etc. These polymerizing agents may be used with or without mild heating. The polymerized substance is then freed from them by washing with water. Polymerization of the semi-drying oils, such as whale oil, may be accomplished by heating, or heat while blowing with air, and by heat in the presence of certain metals, such as magnesium. The same will apply to the hydroxy fatty oil, such as castor oil.

The amount of isocolloid compounded with the lubricating oil will depend somewhat on the viscosity desired. The more isocolloid present, the higher the viscosity tends to be. Theoretically, sufficient isocolloid should be present to form an adsorbed film on the bearing surfaces. In practice, one will add only as much isocolloid as seems to add to the lubricating value or slipperiness. The examples given have proved satisfactory.

In general, it may be stated that to the lubricant base having a polymer isocolloid dispersed therein there is added sufficient thinning agent to substantially reduce viscosity. Preferably 60 to 70% of the thinning agent, such as solvent naphtha, mineral naphtha, turpentine, or other volatile solvent of low viscosity is added. However, it is of course obvious that this may be varied and still come within the spirit of the present invention.

If desired, the lubricants herein set forth may have their viscosity reduced by the addition of an oil of low viscosity. For example, there may be added to the lubricant loom oil which is a hydrocarbon, usually of petroleum origin, of fairly high boiling point, but low viscosity. Loom oil may be added when it is desired to add a large quantity of colloid in proportion to the lubricant, as a larger quantity of colloid may be added because of the low viscosity of the loom oil as compared to the more generally used lubricants. Loom oil, however, has the disadvantage that it is very much inferior in lubricating quality compared to the more viscous hydrocarbons.

As stated, only a small proportion of the polymerized material isocolloidal with the original material is added thereto. In general, it may be stated that satisfactory results are obtained by adding up to 5% or more of the polymerized material. However, the percentage may obviously be considerably varied according to the ingredients and purpose and still be within the spirit of the present invention.

The amount of polar material added will obviously vary in accordance with the physical and chemical characteristics of the original lubricant. However, it may be stated, as a general proposition, that about 1 to 7% of the polar material is added to the hydrocarbon oils. Here again it is obvious that these limits may be considerably varied and come within the spirit of the present invention. In other words, it is specifically desired to point out that the invention is not lim-

ited to the particular polar percentage range set forth.

The present application is a continuation-in-part of application Serial No. 460,545, filed June 11, 1930.

What I therefore claim and desire to secure by Letters Patent is:—

1. A substantially homogeneous lubrication product of penetrative character and relatively low viscosity consisting of a lubricating oil comprising largely hydrocarbons of the class including the paraffin, olefin and naphthene series and containing at least fourteen carbon atoms and polymers of such oils colloidally dispersed in them, and a volatile solvent in an amount sufficient to reduce the viscosity of the combined oil and polymers to below that of the oil in which the isocolloids are dispersed.

2. A substantially homogeneous lubrication product of penetrative character and relatively low viscosity consisting of a lubricating oil comprising largely hydrocarbons of the class including the paraffin, olefin and naphthene series and being a mixture of hydrocarbons of generally high molecular weight and polymers of such oils colloidally dispersed in them, and a volatile solvent in an amount sufficient to reduce the viscosity of the combined oil and polymers to below that of the oil in which the isocolloids are dispersed.

3. A substantially homogeneous lubrication product of penetrative character and relatively low viscosity comprising a hydrocarbon lubricating oil substantially devoid of coal tar compounds and in its original state of high lubricating value having dispersed therethrough a relatively small proportion of an isocolloidal polymer thereof together with a thinning agent for the mixture to reduce the viscosity thereof below that of the original lubricant.

4. A substantially homogeneous lubrication product of penetrative character and relatively low viscosity comprising a hydrocarbon lubricating oil substantially devoid of coal tar compounds and in its original state of high lubricating value having dispersed therethrough a relatively small proportion of an isocolloidal polymer thereof, a polar compound acting to modify the acidity or alkalinity of the lubricant, and a solvent for the mixture to reduce the viscosity thereof below that of the original lubricant.

5. A substantially homogeneous lubrication product of penetrative character and relatively low viscosity comprising a hydrocarbon lubricating oil substantially devoid of coal tar compounds and in its original state of high lubricating value having dispersed therethrough a relatively small proportion of an isocolloidal polymer thereof, an anti-oxidant, and a solvent for the mixture to reduce the viscosity thereof below that of the original lubricant.

6. A substantially homogeneous lubrication product of penetrative character and relatively low viscosity comprising a hydrocarbon lubricating oil substantially devoid of coal tar compounds and in its original state of high lubricating value having dispersed therethrough a relatively small proportion of an isocolloidal polymer thereof, an anti-oxidant, a polar compound acting to modify the acid or alkalinity of the lubricant, and a solvent for the mixture to reduce the viscosity thereof below that of the original lubricant.

7. A substantially homogeneous lubrication product of penetrative character and relatively

80

85

90

95

100

105

110

115

120

125

130

135

140

145

150

low viscosity comprising a semi-drying lubricating oil in its original state of high lubricating value having dispersed therethrough a relatively small proportion of an isocolloidal polymer there-  
5 of and a solvent for the mixture to reduce the viscosity thereof below that of the original lubri-  
cant.

8. A substantially homogeneous lubrication product of penetrative character and relatively 10 low viscosity comprising a lubricating oil having an asphaltic base and in its original state of high lubricating value having dispersed therethrough a relatively small proportion of a polymer there-  
15 of consisting of polymerized asphaltic still bot-  
tom residue and a solvent for the mixture to reduce the viscosity thereof below that of the original lubricant.

9. A substantially homogeneous lubrication product of penetrative character and relatively 20 low viscosity comprising a lubricating oil of high lubricating value having dispersed therethrough up to 10% of an isocolloidal polymer thereof and

a volatile solvent for the mixture to reduce the viscosity thereof below that of the original lubri-  
cant.

10. A substantially homogeneous lubrication product of penetrative character and relatively 80 low viscosity comprising a hydrocarbon lubri-  
cating oil in its original state of high lubricating value having dispersed therethrough up to 10% of an isocolloidal polymer thereof, 1 to 7% of a polar compound, and a solvent for the mixture to reduce the viscosity thereof below that of the original lubricant.

11. A substantially homogeneous lubrication product of penetrative character and relatively 85 low viscosity comprising a lubricating oil of high lubricating value having dispersed therethrough a relatively small proportion of an isocolloid 90 consisting of an isomer or polymer of said lubri-  
cating oil and a volatile solvent for the mixture to reduce the viscosity thereof below that of the original lubricant.

SAMUEL CABOT.

25.

100

30

105

35

110

40

115

45

120

50

125

55

130

60

135

65

140

70

145

75

150